

## UNITED STATES PATENT OFFICE

2,120,119

## STABILIZED LUBRICATING OIL

Waldo L. Steiner, Ponca City, Okla., assignor to  
 Continental Oil Company, Ponca City, Okla.,  
 a corporation of Delaware

No Drawing. Application January 20, 1933,  
 Serial No. 652,698

## 12 Claims.

(CL. 87—9)

My invention relates to improved methods for the production and stabilization of high grade lubricating oils and more particularly comprises such stabilized products as new compositions of matter.

In the production of present day lubricants many substances are added to the hydrocarbon oil to contribute one property or another to the finished lubricant. These addition products may cause cloudiness, precipitation or other objectionable characteristics in the finished lubricant. The change may be due to the properties of the addition material, the properties of the oil, or a combination of the two. In some cases the change is evidenced immediately on blending; in others considerable time may be required before the objectionable change is apparent. Generally, the cloudiness or precipitate disappears or goes back into homogeneous solution with the hydrocarbon oil when the lubricant is put into actual service. This reversal of action is no doubt due in part to the influences of temperature, pressure and metal contact experienced in actual lubricating service.

Cloudy oils are difficult to market and may be the source of considerable sales resistance. In fact, it may be the direct cause of marketing failure of a product which should be a market success. The cloudiness or slight precipitate, as a rule, does not impair the lubricating qualities of the lubricant.

I have found that cloudiness usually results from the presence of free organic acids or substances which will react acid in the lubricant. The degree of cloudiness is greatly influenced by the presence of other substances in the lubricant such as sulphur, soaps and the like.

The primary object of my invention is to stabilize lubricants and prevent the formation of a cloud or precipitate.

Another object of my invention is to accomplish this result cheaply and without in any way impairing the desirable lubricating qualities of the lubricant.

Other objects will be apparent to those skilled in the art on reading the following description of my invention.

In general, my invention comprises the addition of organic substances which are basic or alkaline with respect to the hydrocarbon lubricants which have a tendency to cloud or give a precipitate due to their free acid content or content of acidic substances.

The following example is given to clarify my

invention but is not to be considered as a limitation to my invention.

A high film strength free wheeling gear lubricant can be made by the addition of a sulphur base oil and lead naphthenate to a hydrocarbon mineral oil. The percentage of these constituents in the finished lubricant can be varied over wide limits depending upon a number of factors and particularly on the degree of high film strength desired in the finished lubricant. A common characteristic of all of these blends is that on standing (1 to 30 days) a substance insoluble in the hydrocarbon oil separates, and, if not disturbed, will slowly settle to the bottom of the container. The insoluble material which separates is visible and detracts from the sales value of the lubricant. This is particularly true of the bottom portion of the container where the precipitate has concentrated. To my knowledge this precipitate does not impair the lubricating qualities of the oil.

In my study of the insoluble material, I found that it was influenced and dependent on the free acid content of the lubricant. I could greatly inhibit the formation of the insoluble substance by carefully freeing the lead naphthenate of all free naphthenic acids. This is not commercially feasible, since freeing the lead naphthenate of naphthenic acid is very difficult. Furthermore, lead naphthenate will release free acid again until a certain equilibrium between lead naphthenate acid is reached.

The addition of organic bases to the blend tends to neutralize the free naphthenic acid and substantially prevents formation of insoluble material. At any rate, the formation of the insoluble substance is inhibited to a point where it is not a cause of sales resistance.

In practicing my invention I determine by titration the approximate or exact amount of free acid present in the lubricant and sufficient organic base is added to neutralize the determined amount of free acid with about 5 to 50% excess of the base. The acid content of the various constituents of the finished lubricant may be determined in the usual manner and the organic base added to the acidic constituents or blended with the acidic constituents and the mineral oil in one step.

The organic base should be thoroughly incorporated in the lubricant. With viscous lubricants the blending should be done at high temperatures, say up to 200° F. or above, the temperature used depending on the consistency of the mixture and upon the organic base being used.

Organic bases as used in the description of my invention may include such substances as the nitrogen containing organic compounds. Triethanolamine has been found to be entirely satisfactory and better than many of the other organic bases. Diphenylamine may be used. Aniline is not sufficiently basic to be of much value. Nearly all of the secondary and tertiary amines are satisfactory. Some of the substituted primary amines may be used with success.

Since the amount of free acid occurring in the lubricant is usually small, the amount of organic base used is, as a rule, a very small percentage based on the lubricant volume. The exact amount depends upon the results obtained by titration but I have found that it is usually below 1% and ranges between 0.01% and 0.1%.

My invention is not limited to any theories projected but depends entirely on the results obtained.

It is to be remembered that the cloudiness is caused by the formation of a hydrocarbon insoluble precipitate, and that I use the term "cloudiness" in the general sense to indicate both the appearance of a cloud in the lubricant and the formation of the precipitate.

The sulphur base is prepared from a fatty oil and sulphur. Fatty oils as obtained commercially are not absolutely free of acid and the addition of sulphur tends to saponify part of the fatty oils to form fatty acid, so that considerable free fatty acid is usually found in the sulphur base. It may be that a combination of the free fatty acid and the sulphur base with the free fatty acid from the lead naphthenate may cause the difficulty. At any rate when an organic base is added according to my invention, the difficulty is obviated.

Having thus described my invention, what I claim is:

1. A lubricant comprising in combination a hydrocarbon oil, an addition product of acidic nature and a small quantity of an organic base.

2. A lubricant comprising in combination a hydrocarbon oil, an addition product of acidic nature and a small quantity of an organic base containing an amino group.

3. A lubricant comprising in combination a hydrocarbon oil, an addition product which will release an acid and a small quantity of an organic base.

4. A lubricant comprising in combination a hydrocarbon oil, an acid releasing addition product and a secondary amine.

5. A lubricant comprising in combination a hydrocarbon oil, an acid releasing addition product and a tertiary amine.

6. A lubricant comprising in combination a hydrocarbon oil, an acid releasing addition product and a substituted primary amine.

7. A lubricant comprising in combination a hydrocarbon oil, an acid releasing addition product and a diphenylamine.

8. A lubricant comprising in combination a hydrocarbon oil, an acid releasing addition product and a triethanolamine.

9. A lubricant comprising in combination a hydrocarbon oil, lead naphthenate and an organic base.

10. A lubricant comprising in combination a hydrocarbon oil, lead naphthenate and triethanolamine.

11. A non-clouding lubricant comprising a hydrocarbon oil, lead naphthenate and a small quantity of amine.

12. A non-clouding lubricant comprising in combination a hydrocarbon oil, lead naphthenate and a small quantity of diphenylamine.

WALDO L. STEINER. 40